

April 21, 1925.

1,535,059

F. THARALDSEN

PROCESS FOR MAKING LIQUID ZINC FROM BLUE POWDER

Filed June 7, 1923

FIG. 1.



FIG. 2.



Inventor

Filip Tharaldsen

By

Henry Orth Jr.

Attorney

## UNITED STATES PATENT OFFICE.

FILIP THARALDSEN, OF BESTUM, NEAR CHRISTIANIA, NORWAY.

## PROCESS FOR MAKING LIQUID ZINC FROM BLUE POWDER.

Application filed June 7, 1923. Serial No. 644,066.

*To all whom it may concern:*

Be it known that I, FILIP THARALDSEN, a citizen of Norway, and residing at Bestum, near Christiania, Norway, have invented certain new and useful Improvements in Processes for Making Liquid Zinc From Blue Powder, of which the following is a specification.

In known processes for converting blue powder into liquid zinc it has been deemed essential to subject the powder to friction. The general opinion as to the nature of the powder was that it consists of small metal globules covered with a film of zinc oxyd.

10 The purpose of the friction was to cause a grinding of these globules by which the oxyd film would be removed.

The present invention is based on the fact that the nature of the powder is not that of oxyd-covered globules, but that it consists, for the main part, of non-oxydized metal. Therefore the use of friction or grinding gives only poor results as is well known. It is also generally known that the 20 rotating drum usually employed in the process of converting the powder into liquid zinc does not give any considerable friction to the powder, because the inside walls of the drum will almost immediately become slippery from small quantities of liquid zinc separating. This lubricity of the walls will cause the whole mass of powder to remain at rest during the rotation of the drum.

30 My invention consists in the process of separating the non-oxydized metal from the powder by subjecting the latter to a series of shocks, and preferably while it is contained in a rotating drum which is heated as usual.

In order that my process may be readily understood I have illustrated in the accompanying drawing an apparatus adapted to carry out the process and in which—

Figure 1 is a side elevation, and

Fig. 2 is an end view of a rotary drum provided with means for imparting shocks thereto.

The apparatus shown consists of a cylindrical drum 1, provided on its outer periphery with one or more bearing members in the form of bands 2. These bands have an irregular outer surface and are supported on a series of rolls 3, journaled in bearings 4 on opposite sides of the drum. Two 50 of the rolls 3 are fixed on a driving shaft 5 carrying a pulley 6 which may be driven from any suitable driving member, not shown.

The present process does not aim at frictioning the powder and the usual rotating drum is not used to produce friction but only for the purpose of effecting in a simple manner a continuous series of shocks causing settling in the powder mass, during 65 the movement of the drum. The irregular peripheries of the bands 2, during their rotation by the rolls 3 causes a series of shocks to be imparted to the drum in a direction transverse to the axis of rotation of the 70 latter.

I claim:—

1. The process of making liquid zinc from blue powder which comprises subjecting the powder to a revolving action of a 75 rotary heated drum, and imparting a series of shocks to the drum during rotation thereby causing a settling of the non-oxydized metal of the powder.

2. The process of making liquid zinc from 80 blue powder, which comprises subjecting the powder to a revolving action of a rotary heated drum, and imparting a series of shocks to the drum in a direction transverse to the axis of the latter, during rotation, 85 thereby causing a settling of the non-oxydized metal of the powder.

In witness whereof I affix my signature.

FILIP THARALDSEN.